

## UNITED STATES PATENT OFFICE

2,515,184

## AGE HARDENABLE NICKEL ALLOYS

Clarence George Bieber and Mortimer Pierce  
Buck, Huntington, W. Va., assignors to The International Nickel Company, Inc., New York, N. Y., a corporation of Delaware

No Drawing. Application January 13, 1941,  
Serial No. 374,208

5 Claims. (Cl. 75—170)

1

The present invention relates to nickel alloys, and, more particularly, to hardenable nickel alloys possessing an optimum combination of hot malleability and response to heat treatment. It was known that nickel alloys could be rendered hardenable by incorporating in the alloys such amounts of an alloying element exhibiting increasing solubility with rise in temperature that at elevated temperatures the solid alloy dissolved a greater amount of the alloying element than it could retain in stable equilibrium at lower temperatures. The hardening treatment comprised heating such an alloy to a sufficiently elevated temperature to cause at least part of the hardening element to go into solid solution, rapidly cooling the alloy to produce a super-saturated solution of the element in the alloy, and then reheating at a lower temperature to harden the same. Some of these alloys possessed the ability to harden to relatively high hardness by proper heat treatment, but in these alloys the temperature range of hot malleability was so narrow that, from the point of view of commercial production, they were practically unworkable. These alloys also were sluggish to cast and almost unmachinable. When the attempt was made to broaden the temperature range of hot malleability by modifying the composition of the alloy, it was found that the hardenability was greatly reduced when the temperature range of hot malleability was broadened sufficiently to make the alloy commercially hot malleable. Similarly, the hardness was reduced if the composition of the hardenable alloys was modified to obtain good machinability. The art was faced with the outstanding problem of providing nickel alloys exhibiting hot malleability over a wide enough temperature range for commercial production, having high hardness in the hardening condition, and yet being reasonably soft and machinable in the annealed condition.

We have discovered that nickel alloys characterized by an advantageous combination of hot malleability, relative softness in the annealed condition, and high hardness in the heat treated condition can be regularly produced on a commercial scale by the use of at least two elements from the group consisting of aluminum, titanium and silicon in a critical ratio to the nickel content.

It is an object of the present invention to produce hot malleable nickel alloys capable of being hardened by heat treatment to any selected hardness over a broad hardness range.

It is another object of the invention to produce hardenable nickel alloys containing a critical

amount of at least two hardening elements selected from the group consisting of aluminum, titanium and silicon.

A further object of the present invention is the production of nickel alloys having maximum hardness in the aged condition commensurate with satisfactory forgeability, and good machining properties.

The invention also contemplates improved corrosion and wear-resistant articles of manufacture made of certain carbon-bearing nickel alloys containing critical and controlled amounts of aluminum and titanium and being characterized by the ability to retain high properties at elevated temperatures.

The invention further provides improved age hardened carbon-bearing nickel alloys having controlled and critical amounts of aluminum and titanium characterized by improved hot ductility in the commercial hot working range of temperatures and improved mechanical properties in the age hardened condition.

The mechanical properties of the alloys having combinations of the hardening elements contemplated by the present invention are, to a considerable extent, improved by the presence of carbon. The improvement in the mechanical properties attributable to the presence of carbon may be seen from the illustrative but non-limiting examples given in Table I which show the beneficial effect of carbon in amounts less than about 0.5% on the response to heat treatment of high nickel alloys embodying the present invention.

Table I

| Alloy No. | Composition |     |    |     | Brinell Hardness |              |                    |
|-----------|-------------|-----|----|-----|------------------|--------------|--------------------|
|           | Ni          | C   | Al | Ti  | Annealed         | Heat Treated | Increase, Per.Cent |
| 1         | Bal.        | 0   | .4 | 1   | 158              | 293          | 85                 |
| 2         | Bal.        | .20 | .4 | 1   | 164              | 380          | 132                |
| 3         | Bal.        | .20 | .4 | .75 | 158              | 363          | 130                |
| 4         | Bal.        | .30 | .4 | .75 | 172              | 375          | 118                |

The beneficial effect of carbon illustrated in Alloys No. 2 to 4 inclusive, is surprising in view of the known detrimental effect of carbon on nickel alloys containing titanium as substantially the only hardening element. The difference in the effect of carbon on the hardenability of alloys embodying the present invention containing aluminum with titanium as compared with prior alloys containing titanium as substantially the only hardening element is well illus-

trated by the alloys whose compositions are given in Table IA.

Table IA

| Alloy No. | Composition |    |     |       |      |
|-----------|-------------|----|-----|-------|------|
|           | Ni          | Cu | C   | Al    | Ti   |
| 9         | Bal.        | 30 | 0   | 2.93  | .53  |
| 10        | Bal.        | 30 | .20 | 2.93  | .53  |
| 11        | Bal.        | 30 | 0   | ----- | 3.63 |
| 12        | Bal.        | 30 | .20 | ----- | 3.63 |

The presence of 0.20% carbon in Alloy No. 10 improved the hardenability and raised the hardness in the heat treated condition about 60 Brinell numbers above that of Alloy No. 9 which had substantially the same composition as Alloy No. 10 except that it was substantially carbon-free, whereas the same amount of carbon in Alloy No. 12 made it practically non-hardenable by heat treatment and lowered the hardness in the heat treated condition almost 150 Brinell numbers below Alloy No. 11 which had the same composition as Alloy No. 12 except that it was substantially carbon-free.

The comparatively slight response to heat treatment of alloy 12 is believed to be due to the formation of an inert titanium carbide which decreases the hardening efficiency of the titanium or destroys its hardening ability. The fact that the presence of carbon up to about 0.3% increases the mechanical properties of the material containing both aluminum and titanium made in accordance with the present invention is believed to indicate that the inert titanium carbide does not form in an appreciable amount when aluminum is present with titanium, provided carbon is less than about 0.5% and preferably does not exceed about 0.35%. Carbon within the range of about 0.03% to about 0.3% is highly beneficial in alloys embodying the present invention and

lower the ductility somewhat. For free machining nickel base alloys the carbon content preferably is about 0.2% to 0.3%.

The relative amounts of aluminum, silicon and titanium may vary over a range of several percent provided the ratio of the nickel to the hardener content is maintained within the limits defined herein. At least two of the elements of the group consisting of aluminum, silicon and titanium must be present in the nickel base alloy in amounts greater than about 0.25%. The third hardening element may be present in amounts more or less than 0.25%, the essential feature of this invention being that at least two of the hardening elements must be present in amounts greater than about 0.25%. Aluminum and silicon may be used in amounts up to about 8%, preferably not over 5% of either, while titanium should be less than 11% and preferably is employed in amounts less than 2%. From about 0.25% to under 1% the titanium exerts its greatest effect in combination with aluminum and/or silicon. We have discovered that within the preferred titanium range the optimum combination of hot 15 malleability, hardenability and high hardness in the heat treated condition is obtained when the ratio of the nickel to the weighted hardener content as obtained from the formula,

Weighted hardener content =  $Al + 2.3Ti + Si$  is 30 approximately 15, preferably within the range of 13 to 17, and always within the range of 11 to 20. Since the ratio is a quotient, it is immaterial what unit of weight is used to express the content of nickel, aluminum, titanium and silicon. Thus, 35 for example, the amounts of these ingredients in any given alloy may be given in parts by weight, percentage by weight, etc., without changing the ratio. Examples of alloys illustrating the beneficial results obtained in high 40 nickel alloys embodying the present invention are given in Table II:

Table II

| Alloy No. | Composition |     |       |       |        | Brinell Hardness |              |                   | Ni:WHO <sup>1</sup> |
|-----------|-------------|-----|-------|-------|--------|------------------|--------------|-------------------|---------------------|
|           | Ni          | Al  | Ti    | Si    | Others | Annealed         | Heat Treated | Per Cent Increase |                     |
| 3         | Bal.        | 4.0 | .75   | ----- | .20C   | 158              | 363          | 130               | 16.4                |
| 13        | Bal.        | 4.5 | .75   | ----- | .20C   | 164              | 380          | 132               | 14.4                |
| 14        | Bal.        | 4.0 | .50   | ----- | .20C   | 164              | 248          | 51                | 18.4                |
| 2         | Bal.        | 4.5 | 1.0   | ----- | .20C   | 180              | 380          | 117               | 13.7                |
| 15        | Bal.        | 4.0 | ----- | 1.5   | .10C   | 166              | 302          | 82                | 17.2                |
| 16        | Bal.        | 2.0 | ----- | 4.0   | .10C   | 166              | 321          | 93.5              | 15.7                |
| 17        | Bal.        | 4.0 | .35   | 1.0   | .15C   | 166              | 380          | 129               | 16.2                |
| 18        | Bal.        | 4.5 | .35   | 1.0   | .15C   | 182              | 401          | 120               | 15.0                |
| 19        | Bal.        | 4.6 | .25   | 1.0   | .20C   | 173              | 388          | 125               | 15.0                |
| 20        | Bal.        | 5.0 | .30   | .30   | .20C   | 160              | 375          | 134               | 15.7                |

<sup>1</sup> WHO = weighted hardener content.

which contain aluminum and/or silicon with titanium. This entirely different effect of carbon on titanium may be taken to signify that alloys embodying the present novel combination and containing titanium together with one or both of the elements aluminum and silicon differ in kind from prior alloys substantially free of aluminum and silicon, or containing only ineffective amounts thereof. For general applications it is preferred to have carbon present in amounts from about 0.15% to 0.20%, although even higher amounts may be present. If the carbon exceeds about 0.2% precipitation of graphitic carbon may occur. The presence of graphitic carbon greatly improves the machinability of the alloy and is desirable where free machining properties are required, although precipitated carbon tends to

70 The advantageous combination of properties resulting from the presence of aluminum, titanium and silicon in the above-described ratio obtains even when the nickel has been diluted with appreciable amounts of other elements which enter into solid solution with the nickel. Such elements include copper, chromium and iron. Copper may be present in amounts up to about 45%, chromium in amounts up to about 35% and iron in amounts up to about 45%. These elements increase the base hardness, but offset this by diluting the active hardening elements, i.e., nickel, combined with at least two elements from the group aluminum, titanium and silicon. Copper also lowers the melting temperature, thereby narrowing the hot malleable range. Chromium has an effect similar to copper, except that the

base hardness is increased more rapidly. Chromium also increases the recrystallization temperature and the strength and hardness at elevated temperatures. This increase in strength at high temperatures is, of course, accomplished at the expense of high temperature ductility so that the hot malleable range of the chromium-containing alloys is relatively narrower than the chromium-free alloys. The carbon content of the chromium-containing alloys is preferably kept low, e. g., under 0.1%. One of the great benefits to be derived from the present invention is that the disadvantage of a narrow hot malleable range inherent in prior art age hardenable nickel alloys is substantially overcome by using combinations of at least two metals from the group aluminum, titanium and silicon. At the same time the new alloy possess other desirable properties, including relative softness in the annealed condition, high hardness in the heat treated condition, etc. Certain subject matter originally disclosed in the present application has been described in the following divisional applications, all of which were filed on June 7, 1941: Serial No. 397,080 relating to age hardenable nickel-copper alloys; Serial No. 397,081 relating to age hardenable nickel alloys (now abandoned in favor of application Serial No. 477,144 filed February 25, 1943, also now abandoned in favor of the present application); and Serial No. 397,082 relating to age hardenable nickel-chromium alloys (now abandoned in favor of application Serial No. 477,142 filed February 25, 1943 as a continuation-in-part of the present application).

The alloys of the present invention can be heat treated in the same manner as prior age hardenable alloys, e. g., in accordance with the technique developed by Mudge and described in U. S. Patents Nos. 1,755,554 to 1,755,557 inclusive, or in accordance with the process of our prior copending application Serial No. 253,350 (now Patent No. 2,234,955) of which the present application is a continuation-in-part. The alloys can be softened by quenching or rapidly cooling from about 1500° F. In the softened condition the alloys can be subjected to mechanical working and cold deformation, and in this condition the alloys lend themselves readily to forming and machining operations. Where hardnesses higher than those obtainable by precipitation hardening of hot worked material are desired, the material may be cold worked either before or after the age hardening treatment. For example, fine spring wires may be cold drawn after the hardening heat treatment since this procedure develops the higher physical properties obtainable in the material. It also produces finished material with a higher luster than can be developed in material which is heat treated after cold drawing. Finish machining may also be carried out after heat treatment to eliminate any discoloration and warping which occur during the heat treatment. Heat treated material may be subjected to subsequent machining, stamping or other fabricating operations whenever necessary. In the hardened condition the alloys, as those skilled in the art will readily appreciate, are machinable with greater difficulty than in the annealed condition but, if necessary, machining can be performed by the use of carbide type tools.

In the high nickel alloys containing about 90% or more of nickel, we have found it preferable to employ about 4% to 5% aluminum in combination with about 0.25% to 0.75% titanium and

0.5% to 2% silicon. Carbon should be less than 0.5%, preferably from about 0.15% to 0.20%, except that when free machining properties are desired the carbon should preferably be from about 0.2% to 0.3% as indicated hereinbefore. Small amounts of manganese, iron, sulfur, copper, etc., may be present. The following alloy is typical of the preferred high nickel alloys:

|    |          |
|----|----------|
| 10 | 4.42% Al |
|    | 0.38% Ti |
|    | 1.05% Si |
|    | 0.18% C  |
|    | 0.07% Mn |
| 15 | 0.25% Fe |
|    | 0.02% Cu |
|    | 0.005% S |
|    | 93.6% Ni |

The mechanical properties of the alloy of the specific example as hot rolled, as age hardened and in the aged condition after exposure at 800° F. for 16 months are as follows:

| Properties                   | Hot Rolled | Age Hardened | Age Harned and Exposed 16 Months at 800° F. |
|------------------------------|------------|--------------|---------------------------------------------|
| Proportional Limit, p. s. i. | 34,500     | 110,000      | 118,000                                     |
| Proof Stress, p. s. i.       | 37,000     | 122,000      | 134,000                                     |
| Yield Strength, p. s. i.     | 47,000     | 143,000      | 153,000                                     |
| Tensile Strength, p. s. i.   | 110,500    | 200,000      | 208,000                                     |
| Per Cent Elong. in 2".       | 49.5       | 25.0         | 21.0                                        |
| Per Cent Reduction of Area   | 67.0       | 41.3         | 35.1                                        |
| Hardness (Rockwell "C")      | 2          | 41           | 43                                          |

The room temperature properties of the alloy after exposure for 16 months at 800° F. illustrate the remarkable stability and freedom from "overaging" tendencies which this alloy possesses.

The high nickel alloys of the type illustrated by the data in the preceding schedule may be hot worked over the temperature range of about 1400° F. to about 2450° F., preferably within the range of about 2000° F. to 2300° F.

It will be seen from the foregoing description and the specific examples that we have provided nickel alloys combining optimum response to heat treatment with hot malleability. These alloys may be used for various articles of manufacture including rollers and bearing balls, bearing and races therefor, roller chains, drop forgings and tie rods for airplane construction, valve seats and other valve parts, pump rods and the like, pump rod sleeves, pump pistons for high pressures and temperatures, plungers, turbine blades, turbine diaphragm blading, lock washers, screws and nuts, tools, cutting blades and the like, pins and needles, springs and other resilient elements, airplane instrument parts, nozzles for burners, rods, sheets, strip, wire, bars, rolled shapes, etc.

Although the present invention has been described in conjunction with preferred embodiments, it is understood that modifications and variations may be resorted to without departing from the spirit and scope of the invention, as those skilled in the art will readily understand.

We claim:

- An alloy containing at least 90% nickel, 0.15% to 0.2% carbon, 4% to 5% aluminum, 0.25% to 0.75% titanium, and 0.5% to 2% silicon, the amounts of aluminum, titanium and silicon within said ranges being such that the ratio of the nickel content to the sum of the content of aluminum, silicon and 2.3 times the titanium is between 11 and 20.
- An alloy containing 0.15% to 0.2% carbon,

4% to 5% aluminum, 0.25% to 0.75% titanium, up to 2% silicon, and the balance essentially nickel plus small amounts of incidental elements, the amounts of aluminum, titanium and silicon within said ranges being such that the ratio of the nickel content to the sum of the content of aluminum, silicon and 2.3 times the titanium is between 11 and 20.

3. An alloy containing 0.2% to 0.3% carbon, 4% to 5% aluminum, 0.25% to 0.75% titanium, up to 2% silicon, the balance being essentially nickel which constitutes at least 90% of the alloy, the amounts of aluminum, titanium and silicon within said ranges being such that the ratio of the nickel content to the sum of the content of aluminum, silicon and 2.3 times the titanium is between 11 and 20, said alloy having carbon present in the form of graphite which imparts improved machinability.

4. An alloy containing at least 90% nickel, 0.15% to 0.2% carbon, 0.25% to 5% aluminum, at least 0.25% and under 1% titanium, 0.25% to 5% silicon, and the balance iron and incidental elements, the amounts of aluminum, titanium and silicon within said ranges being such that the ratio of the nickel content to the sum of the content of aluminum, silicon and 2.3 times the titanium is between 11 and 20.

5. An alloy containing at least 90% nickel, 0.2% to 0.3% carbon, 4% to 5% aluminum, 0.25% to 0.75% titanium, up to 2% silicon, and the balance iron and incidental elements, the amounts of aluminum, titanium and silicon within said ranges being such that the ratio of the nickel

content to the sum of the content of aluminum, silicon and 2.3 times the titanium is between 11 and 20, said alloy having carbon present in the form of graphite which imparts improved machinability.

CLARENCE GEORGE BIEBER.  
MORTIMER PIERCE BUCK.

#### REFERENCES CITED

10 The following references are of record in the file of this patent:

#### UNITED STATES PATENTS

| Number    | Name          | Date           |
|-----------|---------------|----------------|
| 1,258,227 | Kelley        | Mar. 5, 1918   |
| 1,277,046 | Cooper        | Aug. 27, 1918  |
| 1,350,359 | Cooper        | Aug. 24, 1920  |
| 1,439,865 | Cammen        | Dec. 26, 1922  |
| 1,556,953 | Parr          | Oct. 13, 1925  |
| 1,572,744 | Mercia        | Feb. 9, 1926   |
| 1,587,992 | Spitzley      | June 8, 1926   |
| 1,610,262 | Cooper        | Dec. 14, 1926  |
| 1,623,948 | Fuller        | Apr. 5, 1927   |
| 1,675,798 | Franks et al. | July 3, 1928   |
| 1,684,131 | Franks et al. | Sept. 11, 1928 |
| 2,005,433 | Lehr          | June 18, 1935  |
| 2,048,165 | Pilling       | July 21, 1936  |
| 2,246,078 | Rohn          | June 17, 1941  |

#### OTHER REFERENCES

30 Campbell: "A List of Alloys," 1930, published by Amer. Soc. for Testing Materials, Philadelphia, Pa., page 26.